

## UNITED STATES PATENT OFFICE

1,922,893

## PROCESS OF MAKING LAMINATED GLASS

James W. Kamerer and Earl L. Fix, New Kensington, Pa., assignors to Duplate Corporation, a Corporation of Delaware

No Drawing. Application January 16, 1932  
Serial No. 587,152

3 Claims. (Cl. 49—81)

The invention relates to a process of making the so called laminated or safety glass which ordinarily consists of two sheets of glass cemented to the opposite sides of cellulose nitrate plastic, 5 such as celluloid, which contains about 70% nitro-cellulose and 28% camphor. The present invention relates to the step of cementing the sheets together when a water soluble cement, such as gelatin, casein, gliadin or xericin, is used. 10 Such cements are the most satisfactory of any so far discovered, but the results attained have not been uniformly good, as indicated by exhaustive tests along two lines; namely, break tests, and roof exposure tests. The roof test involves an exposure of the sample to weather 15 conditions over a long period of time, and the break test involves breaking the sample with a metal ball under certain conditions as to weight and drop, which have been more or less stand- 20 ardized. The roof exposure tests develop a certain amount of edge separation with some samples, while in other cases the break tests show poor adhesion. The object of the present invention is to overcome these difficulties and produce 25 a laminated glass which is uniformly free from edge separation and which uniformly shows good adhesion as evidenced by the break tests.

We have found that this result can be secured by properly conditioning the celluloid. Such 30 conditioning involves the regulation and distribution of moisture through the plastic sheet preliminary to the laminating operation. If the moisture content ranges above a certain percentage, which we have determined, edge separation 35 is liable to occur in the finished product, although the break tests of such product are entirely satisfactory. On the other hand, if the moisture content runs below a certain percentage, which we have also determined, the break 40 tests show unsatisfactory adhesion, although no trouble is experienced with edge separation. Further, the moisture must be well distributed through the body of the plastic sheet, so that superficial drying or wetting is not sufficient.

45 We have found that the proper moisture content ranges from about 1.2% to 1.8%. In order to obtain this condition, the sheets are placed in a conditioning room in which the conditions of humidity and temperature are closely controlled.

50 The sheets are spaced apart so that their entire surfaces are exposed and are left in the room for at least 16 hours in order to insure a distribution of the moisture throughout the body of the plastic sheet. As illustrative of the conditions 55 required in order to insure the moisture content of

from 1.2 to 1.8 per cent, the relative humidity of 55% plus or minus five is maintained. A convenient temperature is 70° F. plus or minus five.

It will be understood that under humidity 60 conditions as they exist in the North Atlantic States, remote from the sea board, a considerable part of the plastic sheets will normally have a moisture content lying between the limits specified, but that such content may depart con- 65 siderably from these limits, in some cases, as low as 1%, and in others as high as 2.5%, and that the conditioning is necessary only to insure a proper moisture content during those periods when the atmosphere is either too moist or too 70 dry to hold the percentage of moisture between the desired limits as heretofore pointed out. At times the plastic sheets are too low in moisture under existing atmospheric conditions, but in the location given the plastic will very often, 75 particularly in summer, have too high a moisture content, so that the conditioning step involves a drying out of the plastic to bring it to the desired condition as to moisture content. Further, conditions of storing the celluloid in 80 packs may result in an uneven distribution of moisture through the sheets, the moisture content at the edges differing very substantially from that at the center of the sheets. The long conditioning period equalizes this moisture 85 content so that each increment of the sheet area is conditioned the same with a consequent uniformity of adhesion throughout the cemented area.

The moisture contents heretofore referred to 90 and as set forth in the claims are not, as a matter of fact, absolute contents, but are figured on the assumption that the plastic is bone dry after drying over calcium chloride as a dehydrater. The term cellulose nitrate plastic, 95 as used heretofore and in the claims, refers to the standard type of material comprising approximately 70 per cent of nitro-cellulose and 28 per cent of camphor. The limits for moisture content, as herein recited, may or may not 100 be advantageous with types of celluloid compositions involving departures from the composition above stated.

We claim:

1. A process of making laminated glass, which 105 consists in treating a sheet of cellulose nitrate plastic in an atmosphere controlled as to moisture content for a period of time such as to secure a uniform distribution therethrough of 1.2% to 1.8% of moisture, and then employing 110

a water soluble adhesive to secure glass sheets to the opposite side of the sheet of plastic.

2. A process of making laminated glass, which consists in treating a sheet of cellulose nitrate plastic in an atmosphere controlled as to moisture content for a period of time such as to secure a uniform distribution therethrough of 1.2% to 1.8% of moisture, and then securing sheets of glass to the opposite sides of the plastic sheet by the use of gelatin cement.

3. A process of making laminated glass, which consists in treating a sheet of cellulose nitrate plastic in an atmosphere controlled as to moisture content for a period of time such as to secure a uniform distribution therethrough of 1.2% to 1.8% of moisture, and then securing sheets of glass to the opposite sides of the plastic sheet by the use of casein cement.

JAMES W. KAMERER.  
EARL L. FIX.

85

15 90

20 95

25 100

30 105

35 110

40 115

45 120

50 125

55 130

60 135

65 140

70 145

75 150